

March 17, 1942.

G. S. ROWELL

2,276,594

PROCESS OF PREPARING PRINTING MEMBERS AND PRODUCT THEREOF

Filed Nov. 17, 1939

2 Sheets-Sheet 1



FIG. 1

BY

INVENTOR.  
GEORGE S. ROWELL

*George S. Rowell*  
ATTORNEY.

March 17, 1942.

G. S. ROWELL

2,276,594

PROCESS OF PREPARING PRINTING MEMBERS AND PRODUCT THEREOF

Filed Nov. 17, 1939

2 Sheets-Sheet 2



FIG. 5

FIG. 6



FIG. 2



FIG. 2a



FIG. 2b



FIG. 3



FIG. 3a



FIG. 3b



FIG. 4

INVENTOR.

GEORGE S. ROWELL

BY

George S. Rowell

ATTORNEY.

## UNITED STATES PATENT OFFICE

2,276,594

PROCESS OF PREPARING PRINTING  
MEMBERS AND PRODUCT THEREOFGeorge S. Rowell, Cleveland, Ohio, assignor to  
George T. Trundle, as trustee, Cleveland, Ohio.

Application November 17, 1939, Serial No. 305,015

28 Claims. (Cl. 101—401.1)

This invention relates to a printing member of the planographic type and to a process of making such printing members. The above indicates the general object.

Other objects include the provision of a process of producing an improved planographic printing surface on malleable material, such as the metals aluminum and zinc; an efficient method of producing flexible planographic printing plates or elements from strip or sheet stock; an improved manner of handling sheet or strip stock in the making of flexible printing members; an improved chemical processing treatment of grained planographic printing members; an improved manner of graining metal surfaces for planographic plate production; an improved manner of handling granular material to facilitate the forcible projection thereof onto malleable material to produce a grained surface thereon; an improved manner of controlling the grain or texture of printing surface on planographic printing members; a more economical and effective manner of making, assembling and protecting planographic printing members for storage pending eventual use, and the product or products of the procedures herein described.

A specific object is to produce a grained surface on a suitable base, which surface has greatly improved qualities for enabling the retention of image or character forming means which are receptive to greasy printing media, such as lithographic ink, and further receptive to aqueous solutions on the non-printing portions to render them ink repellent.

Other objects and various specific advantages of the process and product will become apparent from the following description taken in connection with the accompany drawings. The drawings show preferred procedures in graining and otherwise preparing a planographic printing surface on sheet metal in long strip form. Individual sheets or plates would be similarly treated, except in the matter of feeding, which could be by the use of conveyor belts, sheet grippers on supporting drums, etc. Applicability of various features of the invention to the printing art in other ways, as in order to make non-flexible printing members, will be apparent from the exemplary showing.

In the drawings: Fig. 1 is a diagram illustrating the course of a metal-strip through and along instrumentalities employable in carrying out the process; Figs. 2, 2a and 2b are greatly magnified cross-sectional diagrammatic views of surface portions of strips (e. g.) of metal in the

first stage of graining treatment thereof, but varied relative to each other as will be herein-after described; Figs. 3, 3a and 3b are views similar to Figs. 2 to 2b of the strip surface portions after a second stage of graining treatment; Fig. 4 is a magnified exemplary plan view of a small section of grained surface, at two stages of the graining process; Fig. 5 is a plan view, showing a satisfactory arrangement of nozzles for plate stock of average width; and Fig. 6 is a diagram illustrating a device for throwing abrasive as from a nozzle with substantially uniform effective velocity entirely across a strip in the process of being grained by percussive impact of granular material on the strip.

Lithographic printing using flexible printing members, e. g. thin metal strips or sheets (synonymous with plate in the usual sense) requires, particularly for large editions, a grain surface which will have long wearing life from the standpoint of image retention in definite areas and repellent qualities relative to printing fluid in other definite areas. Considerable variation in coarseness and fineness of grain is required for different uses (types of work) but the attribute of strength and long life in retaining the image definitely and fixedly in the image areas and in repelling printing fluid at definite and fixed non-image areas is always desired. The latter is more delicate or critical. The present invention, inter alia, aims to enable as much variation in the type of grain surface as necessary while securing the element of strength, referred to above, irrespective of the type of grain surface required. The metals zinc and aluminum have respective attributes fitting them for use as planographic printing plate materials. Because of their differences in corrosion resistance, hardness, etc., neither metal is ideal for use interchangeably in the different fields. The present invention tends to lend universal utility to these metals for planographic printing and enables the effective use of a greater range of materials in said field, alloys, compositions, etc., not heretofore found practically usable for planographic printing plates.

The above general discussion is principally in respect to graining the plate, which operation can be accomplished continuously on strip as will now be described.

50 In Fig. 1 a supply of strip S is indicated at 1, illustrating for instance, a roll of aluminum or zinc (or any suitable alloy of either with other metals or materials), on an appropriate support. I prefer aluminum (term includes aluminous alloys) over zinc, partly because of its greater

resistance to corrosion and/or oxidation, and partly because it is harder or can be made harder in dense sheet form without becoming brittle at the surface, or at least can be made more resistant to wear and undesired shininess, as by paper friction.

The strip as shown is suitably guided partially around a drum 2 having a uniform cushion surface, as of live rubber, thence across another similarly surfaced drum 3 and partially around the latter, and thence to a chemical processing apparatus, generally designated 4, to be described later.

Two separate steps of the graining treatment are accomplished on the convex faces of the strip as supported on respective drums. The first step is mainly one of raising minute grain projections on the face of the strip adjacent minute depressions cut therein, and for most satisfactory results requires a shorter radius of curvature on the drum. The second step which is mainly to peen and deform the projections, as will later be described, could be carried out effectively with the metal laid or stretched flat. The drum 3 is preferably about twice the size of drum 2. Both steps, however, can be performed effectively while the metal is supported on a single, curved surface as of a single drum or platen; for example a 10" to 12" rubber covered drum, this being the preferred size for this first step.

Beside the drum 2, at the left as shown, is a throwing mechanism or apparatus 5 for abrasive particles or granules, such as crushed sand, flint, aluminum oxide, etc., the type being selected largely according to the desired use for the grained plates, the malleability and hardness of the material, etc. The abrasive can be thrown by fluid pressure, centrifugally or by impact force on the granules, and the term "blast" used, for convenience, herein includes any suitable throwing means. Sharp abrasive granules are projected, as shown, from a nozzle 10 (preferably a battery of nozzles) which in cooperation with a constant well regulated pressure supply source is or are capable of continuously bombarding with abrasive a fairly narrow area circumferentially of the strip but as an ideal condition, with substantially uniform force and abrasive distribution substantially along the entire width of the strip either instantaneously or progressively laterally of the strip. The strip is advanced at a uniform rate during the bombardment, as by continuously turning the drums, or one of them, or by appropriate strip or sheet feeding means not shown. The rate of advance is varied according to the efficiency of the equipment used for causing the bombardment of the strip by the granules.

One manner in which a flat stream of abrasive can be secured by fluid pressure is by propelling the granules through a flat nozzle. Greater uniformity of impact across the strip, when using a conventional nozzle in fixed position, can be secured by projecting the granules first against a deflector set at an angle to the axis of the nozzle. Also, whether or not such deflector is used, the nozzle or nozzles can be moved back and forth across the work either by rectilinear movement without change in angle of projection relative to the work or by pivotal movement of the nozzle for sweeping back and forth across the work as progressively advanced. In either case, rapid lateral movement of the working portion of the spray across the work produces more uniform graining than a slow movement, partly be-

cause this affords a better opportunity for spent granules to get out of the way of oncoming granules, and avoid being embedded into the strip by such oncoming granules. Granules which remain on the work or are embedded in the work after their force is spent lower the quality of product. It is therefore preferable that they be retained at a minimum.

Fig. 6 shows the nozzle 5 or 30 directed toward a deflecting plate 12 set at an appropriate angle relative to the nozzle and the strip S so that the abrasive grains, although emitted from the nozzle in conical form (as in case of a circular orifice) are spread fanwise against the strip to be grained and thus, broadly speaking, are maintained at substantially uniform concentration per unit of area clear across the strip and more nearly at a uniform impingement angle. The deflecting plate 12 is preferably surfaced with high grade preferably hard rubber, so as to be highly wear resistant. The abrasive granules bounce off the deflector with very little loss in velocity and substantially at constant direction for a given relative adjustment of the deflector and nozzle. The deflector may be appropriately curved, further to secure uniform distribution, in accordance with known laws of reflection.

An important feature both in respect to the first and second graining steps is the control of angles of projection of granules against the work as will be more fully explained later. In the throwing apparatus as in Fig. 1 the angle of incidence of abrasive and work (see lines 23 and 24) can be controlled simply by adjustment of the nozzle about a convenient center, as at 13. In Fig. 6 this control can be effected by adjustment of the deflector 12 or the nozzle, or the nozzle and the deflector. Additional guides and deflectors for the abrasive can, of course, be used for purposes of concentration of granules over limited areas on the strip. Lateral movement of the blast across the work can be obtained by continuously oscillating the nozzle about an axis, such as indicated by the line 14.

In performing the first graining operation, the strip is preferably supported on a curved surface of relatively short radius, this having been found much more effective than when the strip is flat or nearly flat. By way of explanation, the preferred angle of incidence between abrasive and work is a narrow acute angle. If the angle is about or nearly a right angle (as with the nozzle pointing at the drum axis) the surface of the strip is indented, but no proportionate high rims or peaks (terms used interchangeably with projections herein) are raised adjacent the indentations; undesirable permanent embedding of abrasive granules in the strip is apt to occur, and spent granules tend to oppose the action of oncoming granules (buffer action), thus reducing efficiency. In my process, indentations are made but one of the outstanding characteristics of the first step is the throwing up of a comparable and usually greater number of projections above the eventual working surface of the strip or plate. With the strip or plate lying in curved form where worked upon, it is possible practicably to reduce the impingement angle nearly to zero. It is found that, with the work maintained in curved form, spent granules are more effectively discharged and prevented from becoming embedded in the work by oncoming particles. For the best results, especially for use with the finer classes of work, it is desirable that the angle should not approach zero to an extent

such that the abrasive tends to plow parallel furrows. However, such an application, even though producing furrows, does not defeat the purpose as will become clear in connection with the description below of the second step (or series of steps) of the process.

The abrasive is preferably controlled as to size, sharpness, velocity, and angle of projection against the work. In the first graining step, large granules of abrasive may be used for work requiring placement of the image as by lithographic crayon and generally for work requiring a coarse screen effect, e. g., poster work. Finer abrasive, properly controlled, ordinarily results in finer graining, suitable for example in fine screen photo-mechanical process work. Variation from coarse to fine graining with granules of constant size and abrasive quality can also be had by decreasing the velocity. Generally speaking, the deeper a given size of granule is forced into the work the coarser the grain effect will be on the work. Thus, coarse graining can be effected with fine sharp granules by increasing the velocity of impingement of the granules against the work. Conversely, fine graining can be produced with coarse sharp granules. Thus, the ultimate result depends largely upon the velocity at which the granules strike the work, upon the angle of incidence of the granules with the work, and upon the sharpness of the granules. A few illustrations will suffice to show the possibilities for variations in the grain effect obtainable in the first step.

For convenience, projection of abrasive approximately toward the axis of the drum on which the strip stock is supported (trajectory assumed as straight lines) will be referred to as projection at a "direct" angle, and projection toward areas considerably at one side of said axis as at a "meeting" angle.

Fig. 2 illustrates approximately the result of rapid projection of fine sharp granules about midway between a direct and the narrowest practicable meeting angle. Here, P is the normal (untreated) surface of the stock (extended for comparison as at p). Narrow pockets or indentations V are formed and relatively high, closely spaced peaks M which rise above the normal or original surface of the stock. The "grained" surface is both indented and raised relative to P. The metal is also probably torn to some extent, but not enough to detach the peaks from the stock. The inclination of peaks is due to the angle of ricochet of the granules. The arrows indicate the angle of impingement of the granules with the work. Zone 46 on Fig. 4 is typical of the relative arrangement of peaks as raised by the first graining step, viewed in plan. The peaks are more or less parallel to each other.

In Fig. 2a, a narrower meeting angle is employed and the peaks are more inclined than in Fig. 2. Also, the pockets V are not as deep.

Fig. 2b illustrates, in a general way, the character of surface resulting from bombardment of the strip with abrasive at a direct or nearly direct angle. The grained surface is deeply pocketed but not raised much around or adjacent the pockets. This is far less satisfactory for my purpose and I do not recommend its use.

Mixtures of fine and coarse abrasive result in superimposition of fine pockets and peaks on deeper and wider apart pockets and peaks thus further increasing the effective plate area and

holding power for image and repellent, as shown at the left in Fig. 3b (zone 48).

Fig. 1 at the left illustrates diagrammatically one manner of controlling the coarseness and fineness of granules, and the velocities of impact on the stock. Here, 15 and 16 represent supply conduits leading from tanks or hoppers supplied, respectively, say with fine and coarse abrasive granules. The conduits have control valves 17 and 18. 19 and 20 are manipulatable parts connected with respective valves and with a control device for altering, e. g., the pressure and speed of propulsion fluid for the abrasive (or the R. P. M. of a throwing wheel if used). 15 In the particular arrangement illustrated, the finer abrasive is admitted full flow (17 fully open) to the nozzle when the part 19 is adjusted for high speed of propulsion of granules, air valve 21 fully open; and coarse abrasive is 20 at full flow (18 fully open) when the propulsive speed is increased as by opening the air valve 22 of the coarse grain feeding portion of the nozzle. Additional adjustment 19a and 20a in the control elements 19 and 20 enables changes 25 in speed of propulsion of the different classes of granules relative to each other, but at full or any desired partial flow of fine and coarse granules. Mixtures of coarse and fine abrasive at any desired proportions are thereby obtainable for superimposition of fine graining on coarse, as above mentioned. 19a and 20a represent adjustments in the connections 19 and 20 so that projection force and volume of abrasive 30 can be varied relative to each other. The arrangement of nozzle units crosswise of the strip 35 can be as indicated on Fig. 5.

The impact velocity of the abrasive granules on the work can in a given installation be governed by control of air pressure as well known 40 in sand-blasting. When a one-half inch round aperture is used in the nozzle and the nozzle is approximately 15 inches from the work, the average air pressure employed is around 10 to 15 lbs. per sq. inch, using up to 850 cu. ft. per minute of compressed air. The pressure used should not be such as would tend to buckle or distort the sheet itself (as distinguished from the surface of the sheet). It has been found that pressures of over 15 pounds can be used on thick 45 plates, but tend to buckle and distort the same metal .005" to .010" thick which is the usual thickness range for small printing machines. Higher impact velocities can be used on thin metal passing over a curved surface without 50 causing buckling and distortion than can be used on the same metal and thickness flat.

The throwing mechanism 30 for the second step of the graining process may be essentially the same as the mechanism 5, and one nozzle alone can be used if properly manipulated. More satisfactory and uniform work can be done 55 by the use of a nozzle or set of nozzles 31 arranged to bombard the strip somewhat inwardly from the periphery of the larger drum 3 as along the line 32, another nozzle or set of nozzles 33 pointed approximately at the drum axis as along the line 34, and another nozzle or set 35 operating nearer the roll periphery (nearly tangent thereto) as along the line 36. All of these nozzles can be arranged to oscillate rapidly back and forth as on pivot axes normal to the drum axis (see lines 37) to give a sweeping fire of 60 blunt granules, or they can be set at different cross fire angles and reciprocated rectilinearly back and forth crosswise of the strip S. The

nozzles 31, 33 and 35 are also adjustable toward and away from the drum axis and are capable of being locked in adjusted positions, for instance in the illustrative positions suggested on Fig. 1. The nozzles are supplied with granular material and pressure fluid in any known or suitable manner, the outstanding difference from the first graining step being that the granular material for the second step is selected for non-abrasive qualities, blunt or generally rounded grains or pellets being used. The size of grain may be varied as in the first graining step, likewise the force of impingement as by control of air pressure or other throwing force.

The action of the granular material on the work in the second graining step, as mentioned above, is a peening action, and, as illustrated by Figs. 3 to 3b, the projections or peaks M on the preliminarily grained surface are deformed (usually hooked) in such manner as to provide greatly enhanced holding power for moisture and in general for hydrophilic material with which planographic plates are usually, if not always, treated at non-printing areas, and greatly enhanced retaining power for image or character forming media on the printing areas.

With photo-litho methods in current use on conventionally grained plates, the sensitized image is held to the plate, largely if not entirely, by "root" portions of the image material occupying the indentations. These roots become more or less bulbous when a conventionally grained plate is treated after graining, as by passing it through steel pressure rolls. A characteristic of plates rolled after graining is that a top plane is established by the presence of plateaus resulting frequently in undesired bared metal at the top surface of the image. It is impossible to roll down a sand-blast or marble grained plate without crushing down and rendering ineffective the higher grain portions, if the lower portions are to be affected at all. With the present process, the bombardment by the second step causes some action on all the preliminarily grained areas irrespective of height of projections. The smaller granules which are always present work on the smaller peaks through the interstices of the larger peaks. The present invention adds to such rooting of the image, as mentioned above, the locking action of the hooked projections, lending greater life and stability to the image, but without tending to expose relatively large areas of metal at the top level of the image.

Fig. 3 shows at 40 (diagrammatically and greatly magnified) the appearance of the grain after the abrasive graining treatment already described (cf. Fig. 2), and at 41 the result of bombardment of the peaks as by blast from the nozzle or nozzles 31. The angle of impingement of the blunt granules is indicated at 32 (cf. Fig. 1). The bombardment at this stage should have less force than that effected by the nozzle or nozzles at 35, otherwise the peaks or raised effects (may be ridges) are likely to be broken off. Granules striking the sides of the peaks will turn the peaks sidewise and those striking centrally of the peaks turn them along the lines of impact. Thus the peaks or fingers raised by the first graining step tend to project in all directions and this effect may be enhanced by cross fire from different nozzles or by sweeping fire from a single nozzle.

Fig. 3a (at the right, zone 43) illustrates the result of projection of blunt granules from a more direct angle, as from the nozzle or nozzles 75

33 along lines 34. Here less pressure is employed than at either nozzle position 31 and 35. Too much bombardment force will crush the peaks down against the body of the strip or break them off. The direct impingement of granules tends further to mat the peaks, criss-crossing in all directions as illustrated at zone 47 on Fig. 4. The result of bombardment as by the nozzle or nozzles 36 which can be set to operate at nearly a tangent to the drum, i. e. level with the strip area worked on, is to level and clean the grain and further crowd the peaks against each other or the curled ends thereof against the surface of the strip overhung thereby, giving the individual fingers and peaks support at two or more points. Greatest bombarding force can be employed in the peening treatment at the final stage i. e. greater than by nozzles 31 or 33.

It will be seen from the above that the range of angles which are employable for the second (peening) step is greater than for the first step. In the first step there is an outer limit in respect to the meeting angle (suggested by the line 23) beyond which the cutting grains ricochet or bounce off the work without producing deep pockets, although effective peaks may be raised by the furrowing action above described. The inner limit is reached when pockets only predominate. In the second step, the angle of projection of the blunt grains against the work is unlimited, assuming proper bombardment force is maintained.

A steady direct angle of fire in the second graining step would not ordinarily be employed as the initial treatment of the peening process, for then a considerable number of granules would strike between groups of peaks or projections and tend to produce dead spots. The tops of the peaks should be gradually turned. It should be emphasized that the peening treatment can all be done with one nozzle on a given width of strip. For instance, on 10" wide stock, three nozzles oscillated rapidly crosswise of the drum axis from lines of fire at 32 to the line of fire at 36 would approach an ideal arrangement.

Fig. 3b (somewhat larger scale than Figs. 2 and 2a) represents at zone 48 the result of bombarding the work during the first step with coarse abrasive material mixed with finer abrasive material (or separately effecting the two operations, fine after coarse). Smaller peaks and hollows M' and V' are thus imposed on the larger peaks and hollows M and V. The zone 49 is typical of the result of bombardment with blunt grains in the second step.

Referring further to Fig. 4, illustrating at 41 the matted and intermeshing effect of the second graining step on the peaks or fingers formed on the work, the peaks and fingers point in countless directions, forming in effect a jungle of tiny, finger-like elements firmly anchored to the base (strip S) and more or less braced by each other and by the underlying base against dislodgment during the further treatment of the plate stock or handling of it.

The principal reason for operating on relatively widely separated portions of the strip to effect the first and second graining treatments will be apparent from Fig. 1. The abrasive material used in the first step (caught as by a collecting receptacle R) can be salvaged independently of the material (blunt grains) used in the second step (caught similarly as at R'). Otherwise, the two materials could only be separated as to size. The material which becomes worn and

blunted in the first stage can be used effectively in the second stage of the process. Crushed sharp sand should not be used in the peening step. Lake sand is very satisfactory, but round or rounded tiny pellets of any nature can be used, for instance, small glass beads or shot.

Those skilled in the art will perceive that the present grained plate in contrast to marble graining has been kept dry, whereas, usually, marble graining subjects the plate forcibly to moisture for forty minutes or more, probably penetrating the pores of the metal with moisture and other foreign matter tending to accelerate oxidation of the finished plate. The dry graining process, described above, necessarily removes oxide scale, etc., leaving the strip or plate in an ideal condition to be treated, so as to render it permanently ready for use without requiring counter-etching. Such treatment can be carried out automatically in the preferred procedure (using continuously fed strip to avoid intermediate handling and marking), as follows:

After the second bombardment of the plate stock S described above, the strip is passed immediately to the chemical processing treatment (station 4, Fig. 1), as to a tank 50 (or spray) of buffer or oxidation and corrosion arresting material. This is preferably an aqueous solution of dipotassium phosphate ( $K_2HPO_4$ ), which, at proper concentration, will, I have found, preserve the grained plate indefinitely against oxidation and other corrosive influences to which the plate is likely to be subjected even when properly stored. The solution can be approximately 60% of  $K_2HPO_4$  of a specific gravity of about 1.7 and a pH value of from 9.9 to 10.3. This has no corrosive action on steel, hence one does not require a glass lined tank. The grained plate (strip if the process is maintained continuous as shown) stays in the liquid a sufficient time for the solution to reach all the interstices resulting from the graining treatment, which time may vary according to the time required properly to grain the strip. Instantaneous immersion is ample where a 60% solution is used, and because the further treatment does not coat or corrode the grain, the immersion time can be increased as much as desired.

Alternatively, I can use the following solution, among others:

|                    | Ounces |
|--------------------|--------|
| Ammonium fluorides | 5      |
| Ammonia            | 3      |
| Water              | 128    |

The second formula is not as effective or as satisfactory in practice, the latter being due in part to the difficulty in avoiding fumes and loss of ammonia by evaporation.

The strip next passes from the tank to dehydrator apparatus such as squeezing and blotting rolls 52, then is washed as by water spray at 54, further dehydrated as at 56, dried as by electrical elements 58, and is then ready for cutting into suitable shapes and sizes for storage or immediate use.

When subjected to the above described chemical, etc., treatment, the planographic plates made from the stock do not require a counter etch if stored for a long period before use as do the usual planographic plates if not used immediately after graining. The strip or plate, after the chemical treatment, is in such condition that it is immune to oxidation by the water cleaning and drying treatment above described and subse-

quent exposure to normal oxidizing atmospheres. The washing does not remove the chemically obtained protective film or buffer on the grained surface. Thus, the process is a considerable improvement over that followed (e. g.) with marble graining, where a counter-etching, as with acids, was necessary to remove oxides etc., followed by washing and drying and accompanying further oxidation during the drying period; it being well recognized that oxidation of metallic surfaces is promoted by the presence of moisture.

Since the plate of this invention is ready at subsequent times after preparation, as above described, for the acceptance of the printing image or characters without further prior treatment, not only is time and expense saved, but use by careless or unskilled operators is not likely to impair sharpness of grain, whereas were a counter etching required to remove oxidation and other deposits, as heretofore necessary in actual practice, the corrosion of the acid bath frequently reduced the holding power of the plate (or, as known in the art, the plate lost "tooth"), either through lack of proper skill or diligence. In the office devices field, the use of acids for counter etching greatly reduces the market, due to the fact that such acids as required are dangerous to persons and personal property; increase employers' liability costs and require special expenditures for plumbing as a means for washing under readily available running water.

Ordinarily, plates are stacked with their grained faces adjacent paper separators, one of the latter for each plate. A considerable saving in production cost can be effected by carrying out the procedure partially shown at the lower right in Fig. 1. This comprises performing the work above described simultaneously on two strips which are brought together, the second finished strip being indicated at S', with both grained and chemically treated faces adjacent as when passed between assembling rolls 60. Simultaneously, and at proper speed, a separating web as of soft paper W is introduced between the grained faces of the strips S and S' as by rolls 61. From this point the assembly of strips and separator web is conveyed to a shear or cutter, shown diagrammatically as blades 62 and 63, and the plates and separators are then stacked as in the pile or tier T adjacent the cutter.

By using the last described step of the process, the manufacturer obviates practically all necessity for frequent handling of plates, as usually required, incident finger marking and waste of time, securing superior and less expensive plates.

I claim:

1. In forming a planographic printing surface on a printing member, the method comprising blasting one face of the member with relatively sharp granules directed toward said face principally at acute angles relative thereto, whereby to raise minute projections on the material of which the surface of the member is composed, then distorting the tops of the projections to cause them to overhang the member in slightly spaced relation thereto.

2. In forming a planographic printing surface on a printing member having a malleable face portion, the method comprising mechanically treating said face portion generally all over the same in a manner to raise minute, closely spaced projections thereon and to form minute indentations adjacent the projections, and then mechanically distorting the free ends of practically

all of the projections toward the member to cause the projections generally to overhang the indentations in spaced relation thereto at substantially the entire portion which was subjected to the first mechanical treatment.

3. In forming a planographic printing surface on a printing member, the method comprising raising above the normal surface of the material of which the member is composed minute projections on said material, and then distorting the tops of the projections over the entire surface which bears said projections to cause the projections to overhang the member in slightly spaced relation thereto.

4. In forming a planographic printing surface on a printing member, the method comprising raising minute projections on the material of which the surface of the member is composed, then bombarding the surface of the member with a forced blast of granular material of such nature that it does not tend to cut the projections, said bombardment being directed laterally of the projections, whereby to distort the projections partially into overhanging spaced relation to the surface.

5. In forming a planographic printing surface on a printing member, the method comprising bombarding the surface of the member with relatively sharp granules at an angle tending to raise projections thereon, and then bombarding the surface of the member with a forced blast in a manner to distort the projections partially into overhanging spaced relation to the surface resulting from the first bombardment.

6. In forming a planographic printing surface on a printing member, the method comprising bombarding the surface of the member with relatively sharp granules at an angle tending to raise peaks thereon, and then distorting the tops of the peaks to cause them to overhang the member in slightly spaced relation thereto.

7. In forming a planographic printing surface on a printing member, the method comprising abrading the surface of the member with sharp granular abrasive material and then bombarding the surface with a forced blast in a manner to distort the portions of the surface raised by the abrasive material but without cutting said portions to any substantial extent.

8. The improvement in forming a planographic printing surface, comprising relatively indenting and raising respective minute areas of malleable stock and then peening the raised areas of the stock to force portions thereof into overhanging but spaced relation to the indentations.

9. The improvement in forming a planographic printing surface, comprising relatively indenting and raising respective minute areas of malleable stock and then blasting the stock to distort the raised areas of the stock to force portions thereof into overhanging but spaced relation to the indentations.

10. The method of graining flexible malleable sheet material to form a planographic printing surface thereon, comprising bombarding one face of the sheet with relatively sharp abrasive granular material while the sheet is supported on a curved surface, and then bombarding said face with relatively blunt or non-abrasive granular material.

11. The method of graining malleable sheet material to form a planographic printing surface thereon, comprising bombarding one face of the sheet with abrasive granular material projected principally at an acute angle toward said face

in a manner to raise peaks thereon, and then progressively bombarding the resultant face with granules projected at an angle to the principal axes of the peaks.

12. The method of graining malleable sheet material to form a planographic printing surface thereon, comprising bombarding one face of the sheet with abrasive granular material in a manner to raise peaks thereon, and then progressively 10 bombarding the resultant face with granules projected in cross fire relationship to each other against the peaks.

13. The method according to claim 12, wherein 15 in the second mentioned bombardment is partly at a narrow acute angle and partly at a less narrow angle.

14. The method of graining malleable sheet material to form a planographic printing surface thereon, comprising obtaining a coarse grain on 20 one face of the sheet by bombarding said face with coarse abrasive, superimposing a finer grain on the coarse grain by bombarding the same with finer abrasive, and then bending the peak portions of the coarse grain into overhanging spaced relation to adjacent portions of the sheet.

15. The method of graining malleable sheet material to form a planographic printing surface thereon, comprising obtaining a coarse grain on 30 one face of the sheet by bombarding said face with coarse abrasive, superimposing a finer grain on the coarse grain by bombarding the same with finer abrasive, and then bombarding with non-abrasive granules the peak portions of the coarse grain to bend the same into overhanging spaced relation to adjacent portions of the sheet.

16. The method of graining malleable sheet material to form a planographic printing surface thereon, comprising progressively moving the material over spaced supporting surfaces, subjecting the sheet to bombardment with abrasive granular material while on one supporting surface, and then subjecting the grain raised by said bombardment to bombardment with blunt or non-abrasive material while on the other surface.

17. The method of graining malleable sheet material to form a planographic printing surface thereon, comprising progressively moving the material over spaced supporting surfaces of different curvatures, subjecting the sheet to bombardment with abrasive granular material while on the supporting surface having the smaller radius of curvature, and then subjecting the grain raised by said bombardment to bombardment with blunt or non-abrasive material while on the surface having the greater radius of curvature.

18. The method of graining malleable sheet material to form a planographic printing surface thereon, comprising bombarding one face 60 of the material with abrasive in a manner to raise peaks thereon which extend generally parallel to each other, and then bombarding the peaks with blunt or non-abrasive granules in such manner that the peaks are bent out of parallelism and generally into overhanging, spaced relation to the sheet.

19. The method of graining malleable sheet material to form a planographic printing surface thereon, comprising bombarding one face 70 of the material with abrasive in a manner to raise peaks thereon which extend generally parallel to each other, and then bombarding the peaks with blunt or non-abrasive granules from a plurality of directions such that the peaks are

bent out of parallelism and generally into overhanging, spaced relation to the sheet.

20. In graining malleable sheet material in forming a planographic printing surface thereon, the process comprising feeding coarse and fine abrasive granules to a common discharge device and bombarding the sheet simultaneously with the same to impose fine indentations on the coarser indentations and raised effects accomplished by the coarse granules.

21. In graining malleable sheet material in forming a planographic printing surface thereon, the process comprising bombarding a face of the sheet with granules directed at an angle approximately normal to the sheet, then bombarding the face with abrasive granules at a narrower angle to raise rim portions and peaks adjacent the indentations formed by the first bombardment, and then bending the rim portions and peaks heterogeneously into overhanging, spaced relation to the sheet.

22. In graining malleable sheet material in forming a planographic printing surface thereon, the process comprising graining the sheet in a manner to raise minute projections thereon, then bombarding the projections first with raking fire of non-abrasive granules at relatively high velocity and then at lower velocity from a more direct angle relative to the area of the sheet bombarded.

23. In graining malleable sheet material in forming a planographic printing surface thereon, the process comprising graining the sheet in a manner to raise minute projections thereon, then bombarding the projections first with raking fire of non-abrasive granules at relatively high velocity, then at lower velocity from a more direct angle relative to the area of the sheet bombarded, and then further bombarding the resultant grain surface with raking fire of non-abrasive granules.

24. In graining malleable sheet material in forming a planographic printing surface thereon, the process comprising graining the sheet to raise minute closely spaced projections thereon and progressively moving the sheet along a predetermined path while projecting non-abrasive granules onto the sheet from a nozzle whose axis moves rapidly back and forth across the path of progression of the sheet.

10 25. In graining malleable sheet material in forming a planographic printing surface thereon, the process comprising graining the sheet to raise minute closely spaced projections thereon and progressively moving the sheet along a predetermined path while projecting non-abrasive granules onto the sheet from a nozzle whose axis oscillates across the path of travel of the sheet so as to vary the impingement angle of the granules at different areas of the sheet.

15 26. A planographic printing member of malleable material having, on one face, closely spaced relatively narrow projections with their free portions bent or hooked toward the general surface of the member and at least partly in spaced relation thereto.

20 27. A planographic printing member of malleable material having on one face closely spaced peaks with their free ends bent toward the said face in various directions, and portions intermediate to their free ends and base portions in spaced relation to the body of the member in overhanging relation thereto.

25 30 35 28. In making planographic printing members, the method of graining comprising projecting a stream of granular material against a deflecting surface set at an angle to the axis of the stream, whereby to redirect the stream and flatten the cross section thereof, and placing the member to be grained in the way of the redirected granular material to grain the member.

GEORGE S. ROWELL.